# EUROPEAN PATENT SPECIFICATION

(11) **EP 1 196 256 B1**
(45) Date of publication and mention of the grant of the patent: **02.07.2003**
(21) Application number: 99917048.3
(22) Date of filing: 07.04.1999
(51) Int. Cl.: B21B 1/26, B21B 1/46, C21D 9/68, B21C 47/28, B21B 45/08, B21C 47/24

(54) **INTEGRATED CONTINUOUS CASTING AND IN-LINE HOT ROLLING PROCESS, AS WELL AS RELATIVE PROCESS WITH INTERMEDIATE COILING AND UNCOILING OF THE PRE-STRIP**
INTEGRIERTES KONTINUIERLICHES STRANGGIESS- UND INLINE WARMWALZVERFAHREN SOWIE ENTSPRECHENDES VERFAHREN MIT ZWISCHENWICKELN UND ABWICKELN DES VORSTREIFENS
PROCEDE DE LAMINAGE A CHAUD EN LIGNE ET DE MOULAGE CONTINU INTEGRE, AINSI QUE PROCEDE CORRESPONDANT AVEC BOBINAGE INTERMEDIAIRE ET DEROULAGE DU PRE-FEUILLARD

(43) Date of publication of application: 17.04.2002
(73) Proprietor: ARVEDI, Giovanni, 26100 Cremona (IT)
(72) Inventor: ARVEDI, Giovanni, 26100 Cremona (IT)
(74) Representative: Adorno, Silvano
(86) International application number: IT9900082
(87) International publication number: WO00059650

(56) References cited:
- WO-A-93/00179
- WO-A-94/29042
- WO-A-97/01402
- WO-A-97/46332
- FR-A- 2 128 496
- US-A- 4 703 640
- US-A- 5 131 134
- PATENT ABSTRACTS OF JAPAN vol. 011, no. 128 (M-583), 22 April 1987 (1987-04-22) & JP 61 269925 A (KAWASAKI STEEL CORP), 29 November 1986 (1986-11-29)
- SCHOENBECK J ET AL: "STAND DER ISP-TECHNOLOGIE UND NEUE ENTWICKLUNGEN" STAHL UND EISEN,DE,VERLAG STAHLEISEN GMBH. DUSSELDORF, vol. 116, no. 11, page 65-73,158 XP000639880 ISSN: 0340-4803
- GINZBURG V B ET AL: "HEAT CONSERVATION BETWEEN ROUGHING AND FINISHING TRAINS OF HOT STRIP MILLS" IRON AND STEEL ENGINEER,US,ASSOCIATION OF IRON AND STEEL ENGINEERS. PITTSBURGH, vol. 63, no. 4, page 29-39 XP002063816 ISSN: 0021-1559
- PATENT ABSTRACTS OF JAPAN vol. 006, no. 105 (M-136), 15 June 1982 (1982-06-15) & JP 57 036013 A (SUMITOMO METAL IND LTD), 26 February 1982 (1982-02-26)
- PATENT ABSTRACTS OF JAPAN vol. 010, no. 187 (M-493), 2 July 1986 (1986-07-02) & JP 61 030224 A (NIPPON STEEL CORP;OTHERS: 01), 12 February 1986 (1986-02-12)

## Description

The present invention concerns an integrated continuous casting and in-line hot rolling process, as well as the relative plant, for the manufacture of ultrathin steel strip in gauges down to 0.6 mm with such characteristics that, for particular uses such as deep drawing for car body parts, the rolled product obtained may replace a cold rolled product

From WO 00/50189 in the name of the same applicant a process and plant are known for the manufacture of a pre-strip from 6 to 15 mm thick starting from a thin steel slab less than 60 mm thick. The process as per the present invention may be used for example downstream of this known process, expressly concerning a coiling and subsequent uncoiling system of the pre-strip 6-15 mm thick, such as to make possible in the subsequent hot rolling step the manufacture of ultrathin gauge coils but with characteristics similar to those of a cold rolled product

In flat rolled steel manufacturing plants the use of temporary product coiling equipment before the hot finishing rolling mill is known, the purpose of which is to separate the low speed part connected with the continuous caster from the finishing mill which instead works at high speed, so as to form coils which can be used as a spare buffer. A typical application is the so-called "coil box" developed by Selco and used both for traditional plants and for so-called mini-mills which use thin slab technology.

As is known, the coil box in substance contains a series of entry rolls for bending and inviting the flat product to coiling, as well as motorized rolls for giving the necessary rotation to the product for the formation-of the coil which in any case occurs freely, without a central core on which to be coiled and without a box shell. The equipment used, however, presents some drawbacks, the first of which is that of not being suitable for very thin gauges, for example of less than 15 mm, in which case there is an actual collapse of the coil. Moreover, the absence of boxing may lead to problems of non-uniform temperature, critical for obtaining the geometrical tolerances required for the hot production of ultrathin gauge (< 1 mm) coils, but with characteristics similar to coils obtained after a further cold rolling step, at least for particular uses.

It is true that patent US 4.703.640 tries to solve these problems by providing a box and the possibility of using a traditional mandrel, and that patent DE 4013582 supplies a possible solution with two coilers, each boxed in a casing, positioned one above the other, but both solutions have problems of technological and technical nature. Problems of the first type are due to the presence of heads and tails necessarily colder than the central part of the strip, which cause difficulties in the subsequent rolling, especially in the case of ultrathin gauges, giving rise in particular to:
- cobbles due to the so-called "refusals" of the rolling stand to accept material the head of which, over a few centimeters, shows temperature differences of several tens of degrees;
- out-of-tolerances of the first and last section of the strip (several metres), particularly important in the manufacture of ultrathin hot coils which can replace cold rolled ones in certain applications; and
- incorrect positioning or "tail climping" of the tail of the material with consequent damage of the same material and the working rolls.

Still with reference to patent DE 4013582, it can be noted that the strip tail being coiled which corresponds to the leading edge in the subsequent rolling, is subjected to a cooling that can reach about 100°C, in this way making the rolling of strips of any gauge, thin or ultrathin (> or < 1 mm) problematical. Moreover, from a technical point of view, the particular positioning of the coilers, placed one above the other, makes maintenance of the lower one difficult, above all in terms of time, some days being needed to disassemble the upper coiler in order to be able to have access to the lower one. In fact, before being able to intervene, it is necessary to wait for the temperature of the refractory to drop to an acceptable level, and before starting production again, the refractory must again be taken to temperature gradually so as not to cause thereto thermal shocks and damages.

Moreover, taking again into consideration the above-mentioned mini-mills for coil manufacture, one of their characteristics is having a particularly adherent layer of scale on the slab surface, as well as rolled-in scale caused by the upstream processes. To eliminate both types of scale, descalers working at pressures of up to 400 bars have been studied, which however have not solved the problem of completely removing the scale and the consequent defects caused by this on the strip surface, composed mainly of longitudinal lozenges due to scale rolled by the rolls into the strip, which in this way results unsuitable for example for the quality standard for the outerly exposed parts of car bodies as per sectorial standards (for example DIN 1623).

WO 97/46332 discloses an integrated continuous casting and in-line hot rolling process to obtain coils of ultrathin strip adapted to replace, for particular applications, cold rolled coils, said process having the features of the preamble of the present claim 1, as well as a plant for carrying out such a process, having the features of the preamble of claim 3. The plant includes a furnace of traditional type, without any means to control possible overheating, that may involve also other process steps, among wich the descaling which, in this case, is conventional.

JP-A-61-269925 discloses a descaling method in hot rolling through plastic stretching of the strip to mechanically break the scale before the conventional descaling by water

The present invention intends to provide an improved process of the type disclosed by WO 97/46332, provided with an induction heating step and a regulation algorithm for the controlled overheating of the pre-strip head and tail which involves the induction heating, coiling/uncoiling and descaling steps, whereby the pre-strip can be rolled in the austenitic, dual step or ferritic fields. This object is achieved with the process of claim 1, while a preferred way of carrying out the process is described in claim 2.

The invention also provides a plant adapted to carry out the above-mentioned process, as claimed in the independent claim 3 and one or more of the claims depending thereon.

These and other aims, advantages and characteristics of the process and relative plant according to the present invention will result more clearly from the following detailed description of a preferred embodiment of the plant, shown as a non-limiting example, with reference to the attached drawings in which:
**Figure 1** is a schematic view of a part according to the present invention of a plant for the manufacture of ultrathin hot rolled coils with cold rolled characteristics, in a section between the roughing and possible heating step, downstream of the continuous caster, and the finishing rolling step;
**Figure 1a** is a schematic, perspective view of a complete plant including the part of Fig. 1;
**Figure 1b** is a schematic view of a possible construction example with two casting lines-and one finishing line;
**Figures 1c and 1d** show sectional views of the coiling/uncoiling device as per the invention, respectively in the coiling and uncoiling step;
**Figures 2 and 2a** show a section of the pre-strip with adherent and rolled-in scale, respectively before and after plastic stretching of the pre-strip provided by the process of the present invention;
**Figure 3** shows a schematic view, in cross section, of a possible mandrel embodiment to be used for the intermediate coiling/uncoiling coiler provided in the plant according to the present invention;
**Figure 4** shows a front view of the mandrel of figure 3, with the central body assembled by interlocking with the two side segments; and
**Figure 5** shows a sectional view taken along the line V-V of figure 4.

The integrated continuous casting and in-line hot rolling process of the present invention for the manufacture of ultrathin coils includes in sequence, between the initial thickness reduction step, partially with liquid core, and the hot finishing rolling, a coiling and subsequent uncoiling step of the pre-strip with a gauge of 6-15 mm, so that it may have the desired characteristics of constant profile and temperature both transversally (between centre and edges) and longitudinally (between head and tail, passing through the centre).

A plastic stretching step follows immediately, which facilitates the elimination of scale in the subsequent descaling step, in this way making it possible in the subsequent hot rolling step to manufacture ultrathin coils in gauges down to 0.6 mm, which, for certain applications, may replace cold rolled ones.

With reference to the drawings, and in particular to fig. 1, the pre-strip 10, downstream of the continuous caster 7 with simultaneous thickness reduction (not represented) and possible subsequent roughing 8, is subjected to coiling/uncoiling in at least one coiler 11 provided by a mandrel 20 which will be better described hereinafter with reference to figures 3-5. Downstream of the coiler 11, or more than one coiler placed horizontally on the same line, a plastic stretching device 12 is provided, composed of a battery of not less than three rolls (upper and lower) 18, such as to perform a stretching of the material. This plastic stretching leads to the breaking of the continuity between the product and the layer of scale covering it, thus making the latter totally removable in the subsequent descaling step 13, for which reason it will not be necessary to adopt very high pressure descalers, as previously stated, combined with traditional-type mini-mills, before entering the finishing rolling mill 14.

It is to be noted that the coiling/uncoiling device may preferably include auxiliary equipment to favour the entry or exit of the pre-strip in correspondence with the openings of the box casing, parallel to the pass-line, so as not to leave the final part of the pre-strip outside the casing.

In particular, with reference to figures 1c and 1d, the coiling device 11 includes, inside an insulated casing 31, a non-expandable fixed mandrel 20 presenting on its periphery a pocket 21 for inserting the head. Wrapper rolls 33, 33' and 33" are also provided, represented in number of three in Figures 1c and 1d, being mounted on an oscillating arm and pushed inwards so as to be in contact with the outer layer of strip coiled both in complete coiling conditions and therefore at the maximum coil diameter, and at the start of coiling, a condition in which these wrapper rolls are practically in contact with the central mandrel 20.

The casing 11 presents two axial peripheral openings 34 and 35, respectively for the entry of the pre-strip 10 to be coiled (Fig. 1c) and its exit when uncoiling (Fig. Id). The two openings 34 and 35 are preferably defined and included between two respective pairs of rolls for favouring the passage of the pre-strip from outside inwards and vice versa.

Suitable means of control cause rotation of a deviating element 36, pivoting on the roller table 1, until it is directed towards the opening 34 so as to invite the pre-strip 10 to enter the device 11 and, pushed by the wrapper rolls 33, 33', 33", to enter, inserting itself into pocket 21, and be held by the mandrel 20 which, rotating anti-clockwise, as shown in Figure 1c, determines coiling on itself.

In correspondence with the opposite opening 35, an element 37, also having an end normally outside the opening, in a retracted position, can be caused to extend until it inserts this end into the opening so as to form the invitation to the tail of the pre-strip 10 to come out at the start of the uncoiling step, as shown in Fig. 1d, with the mandrel 20 rotating clockwise. The deviating or coiling invitation element 36, as also the extendable and retractable element 37 for uncoiling the pre-strip 10, may of course be made in any other equivalent way suitable for this purpose.

With reference to Fig. 1b, the device 11 is provided movable in a parallel direction to its coiling axis along guide tracks 38 represented in cross-section in Figs. 1c and 1d, on which it can be blocked in fixed coiling and uncoiling positions by means of blocking devices 39.

The moving of device 11 may occur both for maintenance reasons and above all for transferring the coil into an uncoiling position different from the coiling one so as to allow various casting and/or roughing lines to be connected with a single heating and finishing line downstream. On each line shown in Fig. 1b by the roller tables 1, 1', there are two subsequent coiling stations, one set back and one set forward, occupied alternately by the respective device 11 during coiling, as indicated by solid line in the drawing, while the representation of the same device 11 by a dashed line indicates the other possible position.

In correspondence with the central roll table 1c, aligned with the finishing mill 14 downstream, there are two possible coiling stations on which the device of line 1 or line 1' is positioned respectively after coiling in the corresponding forward or backward position. Naturally, these positions are connected to each other by means of two pairs of tracks 38. While a strip is being uncoiled in the centre, there can be simultaneous coiling on two side lines in positions on different axes, so as to reach the central uncoiling position without interference.

With reference to figures 2 and 2a, there is a representation of what happens to the adherent scale 15 and the rolled-in scale 16 on a section of pre-strip 10, the latter caused in particular by upstream processes. Plastic stretching, shown in figures 2a by the arrows pointing outwards, causes lengthening, referred to a section of initial length Lₒ equal to:$\text{E =} \frac{{\text{L}}_{\text{l}} {\text{- L}}_{\text{o}}}{{\text{L}}_{\text{o}}}$

Associated with the stretch, indicated by the arrows in figure 2a, which gives rise to this lengthening, is a plastic bending due to the passage through the rolls 18, which leads to the breaking of the adherent scale 15 and the rolled-in scale 16, much less ductile and more fragile than the steel, above all in the temperature range between 600 and 1300°C. Broken in this way, as shown in figure 2a with 15' and 16', the scale is completely removed in a subsequent descaling step 13 downstream of the device 12, so the pre-strip 10 presents itself at the entry to the finishing mill 14 with a surface free of any type of scale. It is therefore possible, after the finishing mill 14, to obtain a product free of surface defects.

It is to be noted that the above-mentioned plastic bending is achieved preferably by also providing a relative penetration movement between the upper and lower rolls 18, such as to produce bending in plastic conditions which ensures a stretching of the material of more than 2%. For this purpose a control system for the position of the rolls 18 and the force impressed by the device 12 can be provided. This control system preferably includes means able to keep stretching of the material within acceptable values (< 0.7%) of length variation, by using a mass flow variation measuring device, obtained by means of two encoders connected to the entry and exit of the device 12.

The process of the present invention also includes, upstream of the coiler 11, a heating step obtained by means of an induction furnace 9, known already for example from patent EP 0415987. Advantageously, according to the invention, a regulation algorithm is provided for the overheating of the pre-strip head and tail, and in particular temperature control which involves the induction furnace, the coiler and the descaler downstream, with the aim of making it industrially and continuously possible to have a pre-strip suitable for rolling in the austenitic, dual step or ferritic fields in order to obtain hot production of coils in gauges of < 1 mm with the qualities of cold rolled ones.

Practical tests have in fact shown that controlled overheating of the head and tail of the strip are of great help in finishing mill rolling for preventing cobbles and obtaining the best product tolerances, especially in the manufacture of ultrathin products (< 1 mm). Moreover, particular strategies for managing the temperature of the coiler and induction furnace heating, combined with controlled cooling introduced by the descaler 13 downstream, represents the ideal solution for the pre-strip obtainable with the process of the present invention to be suitable for traditional austenitic rolling, two-step rolling between AR1 and AR3 or ferritic rolling under AR1 in the finishing mill. This flexibility allows the optimal crystallization form of the pre-strip to be chosen so as to reach the best quality depending on the type of steel to be obtained.

With reference to figures 3-5, a preferred embodiment is shown of a mandrel 20 to be used for the coiler 11. Figure 3 shows in particular the hollow central shaft 21 of the mandrel inside a central body 22 at the sides of which two steel segments 23 are provided, suitably lightened as is the central body 22. The shaft 21 is cooled by water flowing through the axial hole 24 and externally presents a layer of insulation 25 which, limiting the passage of heat between the shaft and the central body 22, reduces to a minimum cooling of the first section of the strip being coiled and corresponding to the uncoiling tail in subsequent rolling.

Figures 4 and 5, above all the first of these, show a preferred embodiment, of interlocking fit, to join the central body 22 to the side segments 23 by means of shaped fasteners 26, 26', which engage thicknesses 27 inserted to allow assembly, without the need for tie-rods or bolts as required in traditional constructions. These were particularly unreliable because of possible breaking of the tie-rods every 2-3 months, considering that the necessary replacement of the broken tie-rods each time led to a downtime of about two days so as to allow cooling of the refractory material and its subsequent heating.

The particular embodiment shown in figures 3-5 not only has the purpose of increasing the reliability of the mandrel and its ease of execution, but also of making countertension possible between the coiler 11 and the downstream equipment, among which the first stand of the subsequent hot rolling mill. This also facilitates the so-called ferritic rolling in a hot rolling mill which, as stated before, can give the same results as those obtainable traditionally in the subsequent step in a cold rolling mill in order to produce coils of certain qualities, in particular in gauges of < 1 mm.

## Claims

1. Integrated continuous casting and in-line hot rolling process, including in sequence, between a step of liquid steel casting and subsequent thickness reduction until a pre-strip of 6-15 mm is obtained, and a finishing rolling step to obtain ultrathin coils down to a gauge of 0.6 mm, a coiling and subsequent uncoiling step of the said pre-strip, whereby the coils, of ultrathin strip thus obtained can replace, for particular applications, cold rolled coils, **characterized by** the fact of also comprising, between the casting step and the pre-strip coiling/uncoiling step, an induction heating step, with a regulation algorithm for the controlled overheating of the pre-strip head and tail which involves the induction heating, coiling/uncoiling and descaling steps, whereby the pre-strip can be rolled in the austenitic, dual step or ferritic fields, said coiling/uncoiling step being followed by a plastic stretching step to facilitate the elimination of scale in a subsequent descaling step.

2. A process according to claim 1, wherein said plastic stretching step is carried out by subsequent concave-convex bending operations of the pre-strip to form contrary directed arcs with relative penetration movements with respect to the pre-strip axis.

3. A plant for carrying out the process of claim 1, including in sequence, along at least one line of passage (1), downstream of a continuous casting machine (7) and a possible subsequent roughing mill (8), upstream of a hot finishing mill (14), coiling and subsequent uncoiling devices (11) for a pre-strip (10) 6-15 mm thick, **characterized by** the fact that said coiling/uncoiling devices (11) are downstream of an induction furnace (9) and are followed by a plastic stretching device (12) for the pre-strip and a descaler (13), there being provided control means of the induction furnace (9) for the overheating of the pre-strip head and tail through an algorithm-based temperature regulation involving the said induction furnace (9), the coiler/uncoiler (11) and the descaler (13) downstream of the device (12), whereby a pre-strip is obtained suitable for rolling both in the austenitic field and in the dual step or ferritic field.

4. A plant according to claim 3, **characterized by** the fact that the said coiling/uncoiling devices (11) include auxiliary equipment (36, 37) to favour the entry and exit of the pre-strip (10) in correspondence with the respective openings (34, 35) of a box casing (31) in parallel with the said line of passage (1).

5. A plant according to claim 3 or 4, **characterized by** the fact that the said coiling/uncoiling devices (11) include in the said box casing (31) a non-expandable mandrel (20) able to bear a countertension with the equipment downstream.

6. A plant according to claim 5, **characterized by** the fact that the said mandrel (20) is composed of a central body (22) and a pair of lateral segments (23) which can be assembled by interlocking fit on the said central body (22) without bolts and/or tie-rods.

7. A plant according to claim 5 or 6, **characterized by** the fact that the said mandrel (20) includes inside this central body (22) a water-cooled shaft (21) with a layer of external insulation (25) towards the said central body (22).

8. A plant according to claim 3, **characterized by** the fact that the said plastic stretching device (12) is composed of a battery of upper and lower rolls (18) in a total number of at least three.

9. A plant according to claim 8, **characterized by** the fact that the said upper and lower rolls (18) are driven with relative movement of penetration between each other, such as to produce bending in plastic conditions which ensures stretching of the material of more than 2%.

10. A plant according to claim 8 or 9, **characterized by** the fact of including a control program of the position of the rolls (18) and the force impressed by them into the pre-strip material (10).

11. A plant according to claim 10, **characterized by** the fact that the said device (12) includes means to control the stretching of the material within a maximum value of 0.7% of variation of the length by means of a mass flow variation measuring system.

12. A plant according to claim 11, **characterized by** the fact that the said mass flow measuring system includes two encoders connected to the entry and exit of the said device (12).

13. A plant according to claim 3, **characterized by** the fact of including two casting/roughing lines (1, 1') and two or more coiling/uncoiling devices (11) for each line, positionable in respective coiling stations, parallel to the corresponding coiling stations on the other line, each device on a line occupying a coiling station in a staggered position, in the feed direction, with respect to the station occupied at the same time by the device (11) on the other line, the said devices being movable in axial direction until occupying the respective uncoiling positions, parallel to each other but not coinciding, on a central heating and finishing line (1c).

14. A plant according to any of claims 5-7, **characterized by** the fact that the said non-expandable mandrel (20) is contained in an insulated external casing (31) and is able to bear coil weights with a specific weight of even > 100 kg/m, being provided with at least three peripheral wrapper rolls (33, 33', 33") mounted at the end of a respective oscillating arm and two auxiliary devices (36, 37) in fixed positions of respectively coiling and uncoiling to favour the entry of the pre-strip (10) into the device (11) and its exit, respectively in correspondence with two openings (34, 35) practiced on the said casing (31) in parallel direction to the axis of the mandrel (20),

15. A plant according to claim 13, **characterized by** the fact that each device (11) is mounted, movable in parallel direction to the axis of the mandrel (20), on pairs of tracks (38).

## Patentansprüche

1. Integriertes, kontinuierliches Gieß- und In-Line-Warmwalzverfahren, welches aufeinanderfolgend zwischen einem Schritt des Gießens flüssigen Stahls und folgender Dickereduzierung bis zum Erhalt eines Vorstreifens von 6-15 mm und einem Schritt des Fertigwalzens zum Erhalt ultradünner Coils bis hinunter auf einen Gauge-Wert von 0,6 mm einen Schritt des Aufwickelns und folgenden Abwickelns des Vorstreifens umfasst, wobei die auf dieser Weise erhaltenen Coils aus ultradünnem Streifen bei bestimmten Anwendungen kaltgewalzte Coils ersetzen können, **dadurch gekennzeichnet, daß** zwischen dem Schritt des Gießens und dem Schritt des Auf-/ Abwickelns des Vorstreifens zusätzlich ein Schritt des Induktionserwärmens mit einem Regulations-Algorithmus für die gesteuerte Überwärmung des Kopfs und des Rests des Vorstreifens umfaßt ist, welcher die Schritte der Induktionserwärmung, des Auf-/ Abwickelns und des Entzunderns mitumfaßt, wobei der Vorstreifen im austenitischen, Dual-Schritt oder ferritischen Bereich gewickelt werden kann, wobei auf den Schritt des Auf-/ Abwickelns ein Schritt des plastischen Dehnens zum Erleichtern des Entfemens von Zunder in einem folgenden Schritt des Entzunderns folgt.

2. Verfahren nach Anspruch 1, wobei der Schritt des plastischen Dehnens durch sich anschließende Vorgänge eines konkav-konvex-Biegens des Vorstreifens zum Bilden entgegengerichteter Bögen mit relativen Penetrationsbewegungen bezogen auf die Achse des Vorstreifens ausgeführt wird.

3. Anlage zum Ausführen des Verfahrens nach Anspruch 1, welche aufeinanderfolgend entlang wenigstens einer Passagelinie (1) stromabwärts einer kontinuierlichen Gießmaschine (7) und einem möglichen, folgenden Vorwalzwerk (8), stromaufwärts eines Fertigwalzwerks (14), Aufwickel- und anschließend Abwickelvorrichtungen (11) für einen 6-15 mm dicken Vorstreifen (10) aufweist, **dadurch gekennzeichnet, daß** sich die Auf-/Abwickelvorrichtungen (11) stromabwärts eines Induktionsofens (9) befinden und von einer Vorrichtung (12) zum plastischen Dehnen des Vorstreifens und einem Entzunder (13) gefolgt werden, wobei eine Steuereinrichtung des Induktionsofens (9) für die Überwärmung des Kopfs und des Rests des Vorstreifens durch eine Algorithmusbasierte Temperaturregulation, welche den Induktionsofen (9), die Auf-/Abwickler (11) und den Entzunder (13) stromabwärts der Vorrichtung (12) umfaßt, wobei ein Vorstreifen erhalten wird, welcher gleichermaßen zum Walzen im austenitischen Bereich und im Dual-Schritt oder ferristischen Bereich geeignet ist.

4. Anlage nach Anspruch 3, **dadurch gekennzeichnet, daß** die Aufwickel-/Abwickelvorrichtungen (11) eine zusätzliche Ausstattung (36, 37) zum Begünstigen des Eintretens und Austretens des Vorstreifens (10) entsprechend der jeweiligen Öffnungen (34, 35) eines Kastengehäuses (31) parallel zur Passagelinie (1) aufweist.

5. Anlage nach Anspruch 3 oder 4, **dadurch gekennzeichnet, daß** die Auf-/Abwickelvorrichtungen (11) im Kastengehäuse (31) einen nichtdehnbaren Dorn (20) aufweist, welcher in der Lage ist, einer Gegenspannung der stromabwärts gelegenen Ausstattung Stand zu halten.

6. Anlage nach Anspruch 5, **dadurch gekennzeichnet, daß** sich der Dom (20) aus einem zentralen Körper (22) und einem Paar seitlicher Abschnitte (23) zusammensetzt, welche am zentralen Körper (22) ohne Schrauben und/oder Spannstangen durch Verschlußpassung montiert werden können.

7. Anlage nach Anspruch 5 oder 6, **dadurch gekennzeichnet, daß** der Dorn (20) im Inneren des zentralen Körpers (22) eine wassergekühlte Welle (21) mit einer Schicht von externer Isolierung (25) in Richtung zum zentralen Körper (22) aufweist.

8. Anlage nach Anspruch 3, **dadurch gekennzeichnet, daß** die Vorrichtung (12) zum plastischen Dehnen aus einer Gruppe von oberen und unteren Rollen (18) mit einer Gesamtzahl von wenigstens drei aufgebaut ist.

9. Anlage nach Anspruch 8, **dadurch gekennzeichnet, daß** die oberen und unteren Rollen (18) mit relativer Penetrationsbewegung zwischen ihnen angetrieben werden, um ein plastisches Biegen zu erzeugen, welches ein Dehnen des Materials um mehr als 2 % sicherstellt.

10. Anlage nach Anspruch 8 oder 9, **dadurch gekennzeichnet, daß** sie ein Steuerprogramm für die Position der Rollen (18) und die Kraft, mit der sie in das Material des Vorstreifens (10) eindrücken, aufweist.

11. Anlage nach Anspruch 10, **dadurch gekennzeichnet, daß** die Vorrichtung (12) eine Einrichtung zum Steuern des Dehnens des Materials innerhalb eines maximalen Streuungswerles der Länge von 0,7 % mittels eines Massendurchsatz-Abweichungsmesssystems aufweist.

12. Anlage nach Anspruch 11, **dadurch gekennzeichnet, daß** das Duchsatzmesssystem zwei mit dem Eingang und dem Ausgang der Vorrichtung (12) verbundene Kodierer aufweist.

13. Anlage nach Anspruch 3, **dadurch gekennzeichnet, daß** zwei Gieß-/Vorwalzlinien (1, 1') und zwei oder mehrere Auf-/Abwickelvorrichtungen (11) für jede Linie vorhanden sind, welche in jeweiligen Wickelstationen parallel zu den entsprechenden Wickelstationen der anderen Linie positionierbar sind, wobei jede Vorrichtung an einer Linie eine Wickelstation in einer in der Zuführrichtung mit Bezug auf die zeitgleich durch die Vorrichtung (11) an der anderen Linie belegten Station verschobenen Position belegt, wobei die Vorrichtungen in axialer Richtung parallel zueinander, nicht aber zusammenfallend bewegbar sind, bis sie die jeweiligen Abwickelpositionen an einer zentralen Erwärmungs- und Abschlußlinie (1c) belegen.

14. Anlage nach einem der Ansprüche 5-7, **dadurch gekennzeichnet, daß** der nichtdehnbare Dorn (20) in einem isolierten äußeren Gehäuse (31) enthalten ist und in der Lage ist, Rollengewichte mit einem spezifischen Gewicht von selbst > 100 kg/m zu tragen, welche mit wenigstens drei Wickelrollen (33, 33', 33") am Umfang ausgestattet sind, welche am Ende eines zugehörigen oszillierenden Arms befestigt sind, und durch zwei zusätzliche Vorrichtungen (36, 37) in festen Positionen des jeweiligen Aufwickeins und Abwickeins, um das Eintreten des Vorstreifens (10) in die Vorrichtung (11) und sein Austreten jeweils zwei Öffnungen (34, 35) entsprechend zu begünstigen, welche am Gehäuse (31) in einer Richtung parallel zur Achse des Dorns (20) ausgeführt sind.

15. Anlage nach Anspruch 13, **dadurch gekennzeichnet, daß** jede Vorrichtung (11) auf einem Paar von Schienen (38) in einer Richtung parallel zur Achse des Dorns (20) bewegbar befestigt ist.

## Revendications

1. Procédé de coulage en continu et de laminage à chaud en ligne intégré comportant, en séquence, entre une étape de coulage d'acier liquide et de réduction d'épaisseur consécutive jusqu'à ce qu'une pré-bande de 6 à 15 mm soit obtenue, et une étape de laminage de finition pour obtenir des bobines ultra-minces ayant un gabarit descendant jusqu'à 0,6 mm, une étape de bobinage et de débobinage consécutive de ladite pré-bande, de sorte que les bobines, constituées d'une bande ultra-mince obtenue de la sorte peuvent remplacer, pour certaines applications, des bobines laminées à froid, **caractérisé en ce qu'**il comporte également, entre l'étape de coulage et l'étape de bobinage/débobinage de pré-bande, une étape de chauffage par induction, à l'aide d'un algorithme de régulation pour le sur-chauffage commandé de la tête et de la queue de la pré-bande impliquant les étapes de chauffage par induction, de bobinage/débobinage et de décalaminage, de sorte que la pré-bande peut être laminée dans les champs austénitiques et à deux étapes ou ferritiques, ladite étape de bobinage/débobinage étant suivie par une étape d'étirage plastique pour faciliter l'élimination de calamine lors d'une étape de décalaminage suivante.

2. Procédé selon la revendication 1, dans lequel ladite étape d'étirage plastique est effectuée par l'intermédiaire d'opérations d'incurvation concave-convexe consécutives de la pré-bande, pour former des arcs dirigés de manière contraire avec des déplacements de pénétration relatifs par rapport à l'axe de pré-bande.

3. Installation pour mettre en oeuvre le procédé de la présente invention comportant, en séquence, le long d'au moins une ligne de passage (1), en aval d'une machine de coulage en continu (7) et d'un laminoir de dégrossissage suivant possible (8), en amont d'un laminoir de finition à chaud (14), des dispositifs de bobinage et de débobinage consécutif (11) pour une pré-bande (10) d'une épaisseur de 6 à 15 mm, **caractérisée en ce que** lesdits dispositifs de bobinage/débobinage (11) sont en aval d'un four à induction (9), et sont suivis par un dispositif d'étirage plastique (12) destiné à la pré-bande et d'un dispositif de décalaminage (13), des moyens de commande du four à induction (9) y étant agencés pour le sur-chauffage de la tête et de la queue de la pré-bande à travers une régulation de température basée sur un algorithme impliquant ledit four à induction (9), le dispositif de bobinage/débobinage (11) et le dispositif de décalaminage (13) en aval du dispositif (12), de sorte qu'une pré-bande est obtenue, adaptée pour être laminée à la fois dans le champ austénitique, et dans le champ à deux étapes ou ferritique.

4. Installation selon la revendication 3, **caractérisée en ce que** lesdits dispositifs de bobinage/débobinage (11) comportent un équipement auxiliaire (36, 37) pour favoriser l'entrée et la sortie de la pré-bande (10) en correspondance avec les ouvertures respectives (34, 35) d'un carter de boîte (30) parallèlement à ladite ligne du passage (11).

5. Installation selon la revendication 3 ou 4, **caractérisée en ce que** lesdits dispositifs de bobinage/débobinage (11) comportent, dans ledit carter de boîte (31), un mandrin non-extensible capable de supporter une contre-tension avec l'équipement en aval.

6. Installation selon la revendication 5, **caractérisée en ce que** ledit mandrin (20) est constitué d'un corps central (22) et d'une paire de segments latéraux (23) qui peuvent être assemblés par l'intermédiaire d'un agencement de verrouillage mutuel sur ledit corps central (22) sans boulon et/ou tige de liaison.

7. Installation selon la revendication 5 ou 6, **caractérisée en ce que** ledit mandrin (20) comporte, dans ce corps central (22), un arbre refroidi à l'eau (21) ayant une couche d'isolant extérieur (25) en direction dudit corps central (22).

8. Installation selon la revendication 3, **caractérisée en ce que** ledit dispositif d'étirage plastique (12) est constitué d'une batterie de rouleaux supérieurs et inférieurs (18) d'un nombre total au moins égal à trois.

9. Installation selon la revendication 8, **caractérisée en ce que** lesdits rouleaux supérieurs et inférieurs (18) sont entraînés avec un déplacement relatif de pénétration les uns entre les autres, de manière à produire une incurvation dans des conditions plastiques qui assurent un étirage du matériau supérieur à 2 %.

10. Installation selon la revendication 8 ou 9, **caractérisée en ce qu'**elle comporte un programme de commande de la position des rouleaux (18) et de la force imprimée par ceux-ci dans le matériau de pré-bande (10).

11. Installation selon la revendication 10, **caractérisée en ce que** ledit dispositif (12) comporte des moyens pour commander l'étirage du matériau dans une valeur maximum de 0,7 % de variation de la longueur, par l'intermédiaire d'un système de mesure de variation d'écoulement massique.

12. Installation selon la revendication 11, **caractérisée en ce que** ledit système de mesure d'écoulement massique comporte deux encodeurs connectés à l'entrée et à la sortie dudit dispositif (12).

13. Installation selon la revendication 3, **caractérisée en ce qu'**elle comporte deux lignes de coulage/dégrossissage (1, 1') et deux ou plus de deux dispositifs de bobinage/débobinage (11) pour chaque ligne, qui peuvent positionnés dans des postes de bobinage respectifs, parallèlement aux postes de bobinage correspondants de l'autre ligne, chaque dispositif situé sur une ligne occupant un poste de bobinage dans une position étagée, dans la direction d'alimentation, par rapport au poste occupé en même temps par le dispositif (11) sur l'autre ligne, lesdits dispositifs étant mobiles dans une direction axiale jusqu'à occuper les positions de débobinage respectives, parallèles les uns aux autres mais ne coïncidant pas, sur une ligne de chauffage et de finition centrale (1c).

14. Installation selon l'une quelconque des revendications 5 à 7, **caractérisée en ce que** ledit mandrin non-extensible (20) est contenu dans un carter extérieur isolé (31), et peut supporter des poids de bobine ayant un poids spécifique > 100 kg/m, muni d'au moins trois rouleaux d'enveloppement périphériques (33, 33', 33") montés à l'extrémité d'un bras oscillant respectif et de deux dispositifs auxiliaires (36, 37) dans des positions fixes respectivement de bobinage et de débobinage pour favoriser l'entrée de la pré-bande (10) dans le dispositif (11), et sa sortie, respectivement en correspondance avec deux ouvertures (34, 35) pratiquées sur ledit carter (31) dans une direction parallèle à l'axe du mandrin (20).

15. Installation selon la revendication 13, **caractérisée en ce que** chaque dispositif (11) est monté, mobile dans une direction parallèle à l'axe du mandrin (20), sur une paire de pistes (38).
